

## UNITED STATES PATENT OFFICE

2,195,600

## METHOD OF SIZING PAPER

Arthur Reilly, Westbrook, Maine, assignor to  
 S. D. Warren Company, Boston, Mass., a corporation of Massachusetts

No Drawing. Application October 15, 1936,  
 Serial No. 105,831

6 Claims. (Cl. 92—21)

The manufacture of paper, and particularly of sized paper containing alkaline filler, forms the subject matter of this invention.

It is well known that the sizing of paper stock containing an alkaline filler (e. g. calcium carbonate) by means of rosin-size presents difficulties not encountered when the filler is an inert material such as clay. The methods customarily effective in making clay-filled paper, that is, the addition to the paper stock in the beating engine or storage chest of relatively small quantities of ordinary rosin-size and alum, either separately, at the same time, or combined by premixing, generally result in the case of paper containing alkaline filler in very slight or no sizing effect.

To obtain sizing in the production of paper containing alkaline filler it is customary to use one or more of the following procedures: (1) the rosin-size is replaced or supplemented by wax-size; (2) sizing or size-restoring agents are applied to the formed paper-web itself; (3) the "minimizing" method is used whereby addition of alum is made to the stock after it leaves the machine-chest and immediately before it runs out on the paper-machine wire. Although such methods are to a greater or lesser degree effective in producing sizing in alkaline filled paper, they are disadvantageous in use owing to adverse effects upon paper qualities other than sizing and/or to increased complexity and difficulty in machine operation.

The desirability is apparent, therefore, of an effective method of sizing alkaline-filled paper by means of rosin-size, in which no involved procedure is required, and by which no desirable quality of the paper is sacrificed. It is accordingly one object of this invention to provide a method of sizing paper containing alkaline filler by means of rosin-size, whereby the usual operations carried out in beater-sizing are sufficient. A further object is to use a protective colloid to prevent, or greatly decrease, the deteriorating action of the alkaline filler upon the rosin-size precipitate. Another object is to produce paper containing alkaline filler and sizing material precipitated from a size containing rosin-soap and a protective colloid. Other objects and advantages will be apparent as the description proceeds.

It is old to use a protective colloid to prevent the curdling of rosin-size by hard water so that upon subsequent precipitation of the size by alum there is produced a much finer size flock than that yielded by curdled size and alum. In such a case, however, the furnish is rendered perma-

nently acidic by the alum, so that once the size has been precipitated by the alum it is thereafter unaffected by the furnish. When alkaline filler is present in the system, however, the condition is changed radically.

The first action of a protective colloid used in rosin-size added to a furnish containing alkaline filler is possibly analogous to that which it gives in the presence of hard water; that is, the size is protected from curdling prior to being precipitated by alum or other precipitant. Any analogy between hard water and alkaline filler ends, however, with the preliminary stage of protection against curdling. For in the case of paper stock containing alkaline filler it is not possible to render the stock permanently acidic without destroying all the alkaline filler. The most that can be done is temporarily to depress the hydroxyl concentration for a matter of minutes. If such alkaline-filled stock sized with unprotected rosin-size and alum is made up into paper during or within a few minutes following the period of transient hydroxyl depression (according to the "minimizing principle"), the paper may have a considerable degree of sizing. On the other hand, if the size-precipitate is allowed to remain for more than a few minutes in contact with the alkaline furnish, its sizing efficacy is greatly lessened by the alkalinity, and for practical purposes, barring the additional use of restoring agents, may be considered to be destroyed. I have found that the size-precipitate can be so formed and protected against loss in sizing efficacy by the use of suitable protective agents in the size that its sizing ability may be retained in large measure while in contact with alkaline filler for a period of at least several hours after precipitation. The protective action of the colloid upon the size-precipitate is distinct from and in addition to its action in preventing initial curdling of the size emulsion. The success I have achieved in sizing alkaline-filled paper by use of rosin-size containing such a colloid is largely due, I have found, to the resistance of the colloid protected size-precipitate against the destructive effect of excess alkaline filler.

In the practice of the invention there is added to a solution or emulsion of rosin-size (i. e. a rosin-soap with more or less free rosin dispersed therein) a quantity of protective colloid (e. g. casein) equal in weight to 4% or more of the weight of the rosin. The so-protected size is mixed in any customary manner with other ingredients going to make up a fibrous furnish for alkaline-filled paper, and the size is precipitated

by a size-precipitant (e. g. an aluminum salt) before the stock is run out on a web-forming device.

The optimum ratio of protective colloid to rosin naturally will vary depending upon the particular colloid used and upon other conditions in the system. In general, however, a colloid to rosin ratio of 1 to 10 is usually effective in producing improved sizing. As the ratio decreases below 1 to 10, the protective action drops rapidly until it becomes negligible at ratios below about 1 to 25. On the other hand, as the colloid-rosin ratio increases above 1 to 10 the protective action increases to some extent. At the same time, however, in the case of some of the agents, casein, for example, the increase in quantity of protective agent has an undesirable tendency to increase the stability of foam in the system. Accordingly, in using those agents that do stabilize the foam, it is ordinarily not desirable to increase the colloid-rosin ratio above 1 to 5, unless an efficient foam-killer is also used in the system. In case the protective agent is one that has no appreciable effect upon foam stabilization (for instance, oxidized starch), it may be used in quantity equal to or greater than the quantity of rosin if desired.

While the protected size and/or alum may be added at any convenient time or at any desired point in the system, provided only that the alum is not wholly consumed by the alkaline filler before contacting the size, it is preferred to add both the protected size and at least part of the alum in the beater, for in such case any objectionable foam contributed to by the use of the protective colloid has a longer time in which to be dissipated.

By the term "rosin-size" as used herein is meant various known sizes in which at least 45% of the rosin present is in a saponified condition. Such sizes include the ordinary rosin-sizes of commerce which consist of sodium or ammonium resinate, with or without unsaponified rosin dispersed therein. Examples of colloidal materials found effective in protecting the sizing material from deterioration by the alkalinity of the furnish are: blood albumen, casein, corn protein, gelatine, glue, locust-bean gum, oxidized starch and soy-bean protein. Naturally these materials are not equally effective. Each, however, is capable of giving a degree of protective action when present in the rosin-size in a concentration falling within the preferred range of 4% to 20% of the weight of the rosin. Dextrine and the gums arabic, ghatti, karaya and tragacanth have been found to be ineffective.

The degree of sizing obtained by the method disclosed naturally will be dependent upon the quantities of size and size-precipitant used, as well as upon the degree of hydration of the fiber and the proportion of fiber to filler in the furnish, as will be well understood by paper makers.

The following examples illustrate how the invention may be applied:

65

### Example I

A furnish was prepared containing the following materials:

|                   | Parts |
|-------------------|-------|
| Soda fiber        | 125   |
| Sulfite fiber     | 65    |
| Calcium carbonate | 160   |
| Aluminum sulfate  | 5     |

75 This was beaten lightly at 5% consistency.

To each of aliquot parts of this furnish was added rosin-size containing rosin equal to 3% of the weight of the furnish and alum equal to 6% of the weight of the furnish.

The sized furnish was made up into sheets, 5 pressed and dried. The sheets were of approximately 50 lb. basis weight, air-dry. The sheets were made exactly alike except that the rosin-size used (a sodium resinate emulsion containing about 40% of its rosin in unsaponified form) for 10 different sheets contained different protective agents. In each case the protective agent amounted to 10% of the weight of the rosin present.

The resistance to ink penetration by the ink 15 flotation test, and comparative resistance to feathering when written upon with pen and ink, are shown in the following table:

| Protective agent                                               | Seconds<br>sizing<br>by ink<br>flootation |              | Writing resistance |              | 20<br>25     |
|----------------------------------------------------------------|-------------------------------------------|--------------|--------------------|--------------|--------------|
|                                                                | Felt<br>side                              | Wire<br>side | Felt side          | Wire side    |              |
| None                                                           | 2                                         | 2            | Poor               | Poor         | Poor         |
| Casein (dissolved by ammonia)                                  | 8                                         | 7            | Fair               | Fair         | Fair         |
| Oxidized sago starch (low viscosity) (dissolved by hot water)  | 7                                         | 6            | Fair to good       | Fair to good | 30           |
| Oxidized corn starch (high viscosity) (dissolved by hot water) | 12                                        | 8            | do                 | do           | Do           |
| Locust bean gum (dissolved by hot water)                       | 11                                        | 8            | Fair               | Fair         | Fair         |
| Corn protein (dissolved by ammonia)                            | 12                                        | 9            | Fair to good       | Fair to good | 35           |
| Blood albumen (dissolved by cold water)                        | 8                                         | 6            | Fair               | Fair         | Fair         |
| Gelatin (high-grade) (dissolved by hot water)                  | 13                                        | 10           | Good               | Good         | Good         |
| Animal glue (low-grade) (dissolved by hot water)               | 7                                         | 7            | Fair               | Fair to good | Fair to good |
| Soy bean protein (dissolved by ammonia)                        | 10                                        | 6            | Fair to good       | Good         | 40           |

### Example II

A furnish was mixed in the beater in the following order:

|                                                   | Pounds |
|---------------------------------------------------|--------|
| Soda fiber                                        | 1260   |
| Sulfite fiber                                     | 285    |
| Starch (cooked)                                   | 35     |
| Protected size containing:                        | 50     |
| Rosin (as sodium resinate 60% and free rosin 40%) | 18     |
| Casein (dissolved by ammonia)                     | 2      |
| Aluminum sulfate                                  | 40     |
| Calcium carbonate                                 | 570 55 |

Later 12 pounds more of alum was added to the machine chest.

The paper was run out on a Fourdrinier wire and pressed, dried and calendered as usual to 60 give 60 lb. paper (25 x 38—500).

| Sizing test                    | Wire side  | Felt side  |
|--------------------------------|------------|------------|
| Ink flotation                  | 70 seconds | 68 seconds |
| Pen and ink writing resistance | Excellent  | Excellent  |

### Example III

The following furnish was prepared:

|                                    | Pounds |
|------------------------------------|--------|
| Sulfite fiber                      | 855    |
| Soda fiber                         | 380    |
| Broke containing calcium carbonate | 290    |
| Aluminum sulfate                   | 10     |
| Starch (cooked)                    | 50 75  |

To this mixture, after beating but before dropping from the beater, was added:

|                              | Pounds |
|------------------------------|--------|
| Calcium carbonate            | 456    |
| 5 Protected size containing: |        |
| Rosin (all sodium resinate)  | 44     |
| Casein (dissolved by borax)  | 4      |
| Aluminum sulfate             | 30     |

Later 70 lbs. of aluminum sulfate was added  
10 in the machine chest.

The furnish was made up in the usual way into  
55 lb. paper (25 x 38—500).

The sizing by ink flotation was 103 seconds on  
the felt side.

15 *Example IV*

The following furnish was mixed in the order  
shown:

|                                                        | Pounds |
|--------------------------------------------------------|--------|
| 20 Sulfite fiber                                       | 400    |
| Soda fiber                                             | 1000   |
| Broke (coated paper)                                   | 500    |
| Aluminum sulfate                                       | 50     |
| Calcium carbonate                                      | 1600   |
| 25 Protected size containing:                          |        |
| Rosin (as ammonium resinate 50%<br>and free rosin 50%) | 80     |
| Casein (dissolved by ammonia)                          | 9½     |
| Aluminum sulfate                                       | 80     |

30 No additions were made after the beater was  
dumped.

The furnish was then made up into 50 lb.  
paper in the usual way. By the flotation test  
the paper on the felt side showed 46 seconds  
35 sizing.

By the method here disclosed in which rosin-  
size containing a protective agent equal to at  
least 4% of the weight of the rosin is precipi-  
tated in a fibrous furnish going to make paper  
40 containing alkaline filler, and in which the size-  
precipitate is protected against the hurtful ef-  
fect of the alkaline furnish by the said protec-  
tive agent, paper is produced having sizing qual-  
ity markedly superior to that obtainable under  
45 the same conditions without the use of the protec-  
tive agent. The customary routine of paper  
making can be followed without requirement of  
special equipment or special control methods.  
The sizing produced is reliable and satisfactory  
50 for many purposes.

The paper product is characterized as indi-  
cated above in that it is a paper containing an  
alkaline filler, an aluminum resinate and/or  
alumina-resin combination size, i. e. a sizing ma-  
55 terial derived chiefly from a rosin soap and alum  
or its equivalent, and a protective colloid.

It is generally conceded that in making ordi-

nary papers (i. e. papers containing no reactive  
filler) saponified rosin is more effective than me-  
chanically dispersed rosin in imparting sizing.  
Although authorities disagree as to the exact  
mechanism of sizing, it is probably true that sa-  
ponified rosin when acted on by an aluminum  
salt is precipitated as aluminum resinate and/or  
as an association of minute rosin particles ad-  
sorbed upon aluminum hydroxide or alumina,  
said adsorption being more intimate and effec-  
tive than is possible to achieve with rosin mere-  
ly mechanically dispersed.

In furnishes containing alkaline filler, unless  
protected, aluminum resinate is not formed, and  
if added as such it is destroyed and the effective  
association of rosin and alumina is deleteriously  
affected by the alkalinity to the point that sizing  
is substantially destroyed. The effect of the  
colloid in the present invention is that the col-  
loid by its presence makes possible the forma-  
tion of aluminum resinate and keeps the pre-  
cipitate stable, and further protects the rosin  
alumina association from the harmful effect of  
alkalinity. Consequently paper made by this  
method retains, and in effective form, the colloid  
25 protected aluminum resinate and/or rosin-  
alumina association, substantially unaffected by  
the action of the alkaline filler.

I claim:

1. Method of sizing paper containing alkaline 30  
filler which comprises forming a furnish com-  
prising fibrous material, alkaline filler, a rosin  
size precipitant and a rosin size at least 45% of  
the rosin content of which is saponified, said  
rosin size containing a protective colloid of the 35  
group consisting of blood albumen, casein, corn  
protein, gelatine, glue, locust bean gum, ox-  
idized starch and soy bean protein in quantity  
amounting to at least 4% of the weight of rosin  
in the rosin size.

2. Method as defined in claim 1 in which the  
protective colloid is casein.

3. Method as defined in claim 1 in which the  
protective colloid amounts to from 4 to 20% of  
the rosin content of the rosin in the size.

4. Method as defined in claim 1 in which the  
ratio of protective colloid to rosin in the rosin  
size is at least 1 to 10.

5. Method as defined in claim 1 in which the  
ratio of the protective colloid to the rosin in 50  
the rosin size is from about 1 to 10 to about 1  
to 5.

6. Method as defined in claim 1 in which the  
protective colloid is casein in quantity amount-  
ing to at least 4% of the rosin content of the 55  
rosin size and the size precipitant is alum.

ARTHUR REILLY.